

3,208,938

## LUBRICATING COMPOSITIONS

Hyman Ratner, Florissant, Mo., assignor to Shell Oil Company, New York, N.Y., a corporation of Delaware  
No Drawing. Filed Feb. 8, 1963, Ser. No. 257,067  
15 Claims. (Cl. 252—32.5)

This invention relates to improved hydrocarbon lubricants and particularly to mineral lubricating oil compositions which possess good detergency, antiwear, as well as sludge, corrosion or rust inhibiting properties.

It is known that certain non-ash forming polymeric nitrogen-containing compounds in which the nitrogen-containing groups may be amino or amido groups such as vinyl pyridines or vinyl pyrrolidones, function as detergents when added in small amounts to lubricants such as mineral lubricating oils. However, copolymers of this type have been found to lack wear inhibiting properties and are corrosive and under severe conditions of use such as under extreme temperatures and pressure they have been found to be shear unstable resulting in sludging and other undesirable side effects.

In order to overcome these defects, the art discloses that the addition of basic polyvalent metal salts such as basic alkaline earth metal petroleum sulfonates or aromatic carboxylates such as alkyl salicylates, impart wear inhibiting and anti-scuffing properties to lubricants containing the above-mentioned non-ash forming detergents. However, it has been observed that the problem of corrosion remains and undesirable side effects such as sludging arises due to the apparent complexing tendencies between the nitrogen-containing polymer and the basic metal salts.

It has now been discovered that excellent ash-free detergent lubricants are provided having in addition wear and corrosion inhibiting properties as well as being resistant towards sludging tendencies, by dispersing in lubricating oil compositions such as mineral lubricating oils containing polymer nitrogen-containing detergents, a small amount of an oil-soluble complex of a polyamide and an acidic compound selected from the group consisting of an alkyl acid phosphate and an alkyl phenoxy carboxylic acid, the complex having the general formula:



where R is an alkyl radical of 8 to 22 carbon atoms, n is an integer of 1 to 10, R' and R<sub>1</sub> are hydrogen or C<sub>1-4</sub> alkyl radicals and (A) is the acidic compound alkyl acid phosphate having the formula:



or



where R<sub>2</sub> is a hydrocarbyl radical, e.g. C<sub>1-6</sub> alkyl or chloroalkyl radical, R<sub>3</sub> is a hydrocarbyl radical such as an alkyl, aralkyl, cycloalkyl radical having from 1 to 18 carbon atoms, X is selected from the group consisting of oxygen and sulfur, m can be zero or one, y is an integer of from 1 to 5 and x in Formula I is 1 or 2.

The detergent nitrogen-containing polymers useful in compositions of the present invention include copolymers of monomers having polymerized linkages and containing nitrogen containing groups which may be amino or

amido groups. They may be derived from polymerizable monomers containing primary, secondary or tertiary (the latter two are preferred) amino nitrogen, including heterocyclic amino or amido nitrogen-containing substances, having an ethylenically unsaturated polymerizable group. These detergent polymers may be obtained by polymerizing vinyl substituted heterocyclic nitrogen-containing substances such as vinyl pyridine, vinyl picoline and vinyl quinoline, vinyl pyrrolidone or vinyl arylamines such as 5 paraaminostyrene, or polyamines prepared by reacting polymeric epoxy compounds with ammonia or primary or secondary amines, with polymerizable unsaturated alcohols, acids or esters such as acrylates and methacrylates of long chain fatty acids, and the like. The preferred polymeric amino or amido compounds are those containing tertiary amine groups and particularly those containing heterocyclic amino groups such as obtained by copolymerizing a polymerizable heterocyclic nitrogen base compound with a polymerizable unsaturated material free of heterocyclic nitrogen-containing radicals such as are described in British patent specification 760,544 and U.S. Patents 2,839,512 and 2,889,282. The copolymers include: copolymer of stearyl methacrylate, and 2-methyl-5-vinyl pyridine; copolymer of stearyl methacrylate, lauryl methacrylate and 2-methyl-5-vinyl pyridine; and those which contain additional C<sub>1-4</sub> alkyl methacrylates in the polymer, such as copolymers of stearyl methacrylates, lauryl methacrylate, methyl methacrylate and 2-methyl-5-vinyl pyridine; and similar copolymers in which the methyl methacrylate is replaced by butyl methacrylate and the 2-methyl-5-vinyl pyridine is replaced by 5-ethyl-2-vinyl pyridine; or copolymer of lauryl methacrylate and N-vinyl pyrrolidone or similar copolymers as described in the British Patent 808,664, and mixtures thereof. Acrylate-vinyl pyrrolidone copolymers are sold by Rohm & Haas under the designations Acryloid 315X or 917 or 966 and are copolymers of N-vinyl pyrrolidone and lauryl methacrylate of varying molecular weights. Other suitable polymeric amines are those available commercially such as those sold by E. I. du Pont de Nemours and Co. under the designations LOA 564 and 565, which are copolymers of lauryl methacrylate and diethylaminoethylmethacrylate (note U.S. Patent 2,737,496).

Particularly preferred detergent polymers are Acryloid 45 917 and 966 (copolymers of N-vinyl pyrrolidone and lauryl methacrylate in the molecular weight range of 400,000 to 500,000) or the copolymers of vinyl pyridine and mixtures of dissimilar methacrylate esters, the preparation of which is illustrated by the following examples.

## EXAMPLE I

A mixture of 25% of 2-methyl-5-vinyl pyridine and 75% stearyl methacrylate was heated in a 50-50 mixture of benzene and a light mineral oil (East Texas 100 65 SSU at 100° F. neutral) to about 120° C. at which time 0.25% wt. of tert. butyl peroxide was added and the reaction mixture was maintained at this temperature for about 6 hours.

At the completion of the reaction, the solvent was 60 stripped off and the polymer diluted with neutral oil to a polymer content of about 30% by weight and filtered at 100-210° C. The copolymer had a molecular weight of about 500,000 and a nitrogen content of 2.94%.

## EXAMPLE II

30% stearyl methacrylate, 51% lauryl methacrylate, 14% methyl methacrylate and 5.0% 2-methyl-5-vinyl pyridine were charged to a 300-gallon stainless steel autoclave. A 50-50 mixture of benzene and neutral petroleum oil was then added to the autoclave so as to furnish 70 1 part of the mixture per 3 parts of the total monomer.

0.25% of ditert.butyl peroxide was then added and the mixture heated at 120° C. for about 7 hours.

At the completion of the reaction, the benzene was stripped off to final conditions of 120° C. and 10 mm. Hg with nitrogen purging. The benzene-free product was then diluted with neutral oil to a polymer content of about 30% by weight and filtered at 100-120° C. The polymer had a molecular weight of about 600,000 and a nitrogen content of 0.54%.

The molecular weights of the polymers were determined by the light scattering method.

The second essential additive used in compositions of the present invention is the polyamide complex as represented by Formula I. The cationic portion of the complex is prepared by reacting a polyamine such as ethylene diamine, propylene diamine, diethylene triamine, triethylene tetraamine, trimethyl trimethylene diamine, hexamethylene diamine, N-2-aminoethylpiperazine and the like with aliphatic carboxylic acids of from 2 to 22 carbon atoms such as acetic acid, propionic acid, butyric acid, caprylic acid, capric acid, lauric acid, palmitic acid, stearic acid, oleic acid, ricinoleic acid and mixture thereof and comprises reacting approximately equimolecular quantities of a polyamine and a fatty acid at between 120° C. and 250° C. for a period of 10 or more hours, preferably under atmospheric pressure. For example, 1 mole of alkyl substituted diethylene triamine,



and two mols of oleic acid were mixed and heated at 175-200° C. for about 10-15 hours in a closed vessel under atmospheric until the diamide formed, after which the reaction was cooled and the end product has the following formula



where R is oleyl radical. Other diamides include distearyl amide of ethylene diamine, dilauryl amide of diethylene triamine, dioleyl amide of diethylene triamine, diricinoleyl amide of diethylene triamine, dioleylamide of N-2-aminoethyl piperazine and mixtures thereof.

The acid portion of the complex includes hydrocarbyl acid phosphates, e.g. mono and dialkyl, mono and dicycloalkyl, diaralkyl, diaryl, alkyl aryl, aralkyl alkyl acid phosphates and their thio derivatives having from 8 to 30 carbon atoms in the molecule. Examples of suitable mono- and di-acid and/or thio acid phosphates are mono and distearyl acid phosphate, mono and dioleyl acid phosphate, mono and dicyclohexyl acid phosphate, dicesyl acid phosphate, lauryl cresyl acid phosphate, dibenzyl acid phosphate, lauryl benzyl acid phosphate, dilauryl acid dithiophosphate, dilauryl thio acid phosphate; alkyl acid phosphonates such as monobutyl chloromethyl phosphonate, monolauryl chloromethyl phosphonate and the like. A preferred alkyl acid phosphate is "Lorol" acid phosphate, which is a mixture of phosphoric esters of "Lorol alcohol." The term "Lorol alcohol" is used in the trade to denote a mixture of primary normal aliphatic alcohols of 8 to 12 carbon atoms which are obtained by fractionation of the alcohols resulting from the reduction of cocoanut and/or palm kernel oils. "Lorol" acid phosphate mixtures are readily obtainable on the market and for this reason are preferred to the purified esters of greater scarcity and higher price. One "Lorol" acid phosphate type is sold under the trade name "Ortholeum 162" and is understood to be mainly a mixture of the mono and diacid phosphates of "Lorol alcohol."

The other acid portion of the complex can be an  $\text{C}_{1-20}$  alkyl phenoxy carboxylic acid such as nonyl phenoxy acetic acid, nonyl phenoxy butyric acid, stearyl phenoxy acetic acid, nonyl phenoxy propionic acid, and the like.

The complex is prepared by reacting 1 mole of the polyamide with 1 to 2 moles of the acid phosphate and/or alkyl phenoxy carboxylic acid at between 50-200° C. for a period of from 2-10 hours. Thus, about 1 mol of the dioleylamide (Ia)



and 1 mole of a mixture of mono and dilauryl acid phosphate was reacted at 100-150° C. for 5 hours at which time the complexing appeared to be complete and a homogeneous product containing phosphorus was obtained. This complex is identified as (Ib).

Another complex (Ic) was prepared under above described conditions using dioleylamide of N-2-aminoethyl piperazine and a mixture of mono and dilauryl-acid phosphate under conditions described for the preparation of (Ib).

Other complexes include (Id) complex of dioleylamide of ethylene diamine and dilauryl acid phosphate, (Ie) complex of dioleylamide of triethylene triamine and dioleyl acid phosphate, (If) distearyl amide of triethylene tetramine and monobutyl chloromethyl phosphonate. The complexes with alkyl phenoxy carboxylic acids and the polyamines include (IIa) complex of dioleylamide of (Ia) and nonyl phenoxy acetic acid, (IIb) complex of dioleylamide of N-2-aminoethylpiperazine and nonyl phenoxy acetic acid, (IIc) complex of distearyl amide of diethylene triamine and nonyl phenoxy acetic acid, (IId) complex of dioleyl amide of diethylene triamine and nonyl phenoxy butyric acid, (IIf) complex of diricinoleylamide of diethylene triamine and lauryl phenoxy acetic acid and the like.

Although the stability and wear inhibition of various functional fluids such as mineral oils or synthetic lubricants are greatly improved by addition thereto of the complex compounds described, the oxidative stability of such compositions is greatly enhanced and the overall properties of such compositions substantially improved by addition thereto of a small amount (0.01-2% by weight, preferably 0.1-1% by weight) of a methylene bisphenol such as

1,1-bis(2-hydroxy-3-t-butyl-5-methylphenyl)methane; bis(2-hydroxy-3-t-butyl-5-methylphenyl)ethane; 1,1-bis(2-hydroxy-3-t-butyl-5-methylphenyl)propane; bis(2-hydroxy-3-t-butyl-5-methylphenyl)-butane; bis(3-hydroxy-3-t-butyl-5-methylphenylisobutane; 1,1-bis(6-hydroxy-5-t-butyl-3-methylphenyl)methane; bis(2-hydroxy-5-t-butyl-3-methylphenyl)ethane; 1,1-bis(2-hydroxy-5-t-butyl-3-methylphenyl)propane; 1,1-bis(2-hydroxy-5-t-amyl-3-methylphenyl)butane; 1,1-bis(2-hydroxy-5-t-amyl-3-methylphenyl)isobutane; etc.

The referred bisphenol is 4,4'-methylene bis(2,6-ditert-butylphenol).

Minor amounts of each class of additives are sufficient for a highly effective combination. The nitrogen containing copolymer and the complex diamide-phosphate or alkyl phenoxy carboxylic acid may be used in an amount of about 0.1-10%, preferably about 0.2-5% by weight each of the lubricant, while about 0.05-2%, preferably about 0.1-1% of the methylene bisphenol is highly useful.

The additive combinations of the present invention may be used to improve various hydrocarbon lubricating oils, whether of natural origin or synthetic, especially oils which are substantially paraffinic and/or naphthenic; they may contain substantial proportions of hydrocarbons having aromatic character but the amounts and types of components should be such that the Dean and Davis (Chem. and Met. Eng., vol. 36, 1929, pp. 618-619) viscosity index of the base oil is at least 80, preferably at least 90 to 150.

The oil may be derived from a highly paraffinic crude, in which case distillation and/or dewaxing may be sufficient to provide a suitable base stock; a minimum of chemical or selective solvent treatment may be used if desired. Mixed base crudes and even highly aromatic crudes which contain paraffinic hydrocarbons also provide suitable oil base stocks by well known refining techniques. Usually these comprise the separation of distillate fractions of suitable boiling range followed by selective

solvent extraction with solvents such as furfural, phenol and the like to provide raffinate fractions which are suitable for further refining by dewaxing and chemical treatment such as sulfuric acid treatment, etc. Thus, it may be a refined hydrocarbon oil obtained from a paraffinic, naphthenic, asphaltic or mixed base crude, and/or mixtures thereof, such as SAE 5W, 10W, 20W, 20, 30, 40, 50 mineral oils. The hydrocarbon oils may be blends of different mineral oil distillates and bright stock; they may have blended therewith a minor but compatible proportions fixed oils, such as castor oil, lard oil and the like and/or with synthetic lubricants, such as polymerized olefins, e.g., polyisobutylene.

The following compositions are representative of the invention.

**Composition A:** Percent

|                                              |         |
|----------------------------------------------|---------|
| Complex Ib                                   | 1.4     |
| Ex. I polymer                                | 5.0     |
| Bis(3,5-ditert.butyl-4-hydroxyphenyl)methane | 0.5     |
| Mineral lubricating oil (SAE 30)             | Balance |

**Composition B:**

|                                              |         |
|----------------------------------------------|---------|
| Complex Ic                                   | 1       |
| Ex. II copolymer                             | 5.0     |
| Bis(3,5-ditert.butyl-4-hydroxyphenyl)methane | 0.5     |
| Mineral lubricating oil (SAE 30)             | Balance |

**Composition C:**

|                                                      |         |
|------------------------------------------------------|---------|
| Complex Id                                           | 1.5     |
| Copolymer of N-vinyl pyrrolidone/lauryl methacrylate | 5       |
| Bis(3,5-ditert.butyl-4-hydroxyphenyl)methane         | 0.5     |
| Mineral lubricating oil (10W-30)                     | Balance |

**Composition D:**

|                                 |         |
|---------------------------------|---------|
| Complex Ib                      | 1.4     |
| Copolymer of Ex. II             | 5.0     |
| Mineral lubricating oil (SAE20) | Balance |

**Composition E:**

|                                              |         |
|----------------------------------------------|---------|
| Complex IIa                                  | 1.5     |
| Copolymer of Ex. II                          | 5.5     |
| Bis(3,5-ditert.butyl-4-hydroxyphenyl)methane | 0.5     |
| Mineral lubricating oil                      | Balance |

**Composition F:**

|                         |         |
|-------------------------|---------|
| Complex of IIb          | 1       |
| Copolymer of Ex. II     | 5.5     |
| Mineral lubricating oil | Balance |

**Composition G:**

|                                              |         |
|----------------------------------------------|---------|
| Complex of Ib                                | 2       |
| Copolymer of Ex. I                           | 5       |
| Bis(3,5-ditert.butyl-4-hydroxyphenyl)methane | 0.5     |
| Mineral lubricating oil                      | Balance |

Other representative non-ash forming lubricating compositions of the present invention include mineral oil containing:

H—2.5% copolymer of Example I+0.5% of Complex IIe

I—2% copolymer of Example II+0.25% of Complex IIId

J—5% of copolymer of stearyl methacrylate/lauryl methacrylate/2-methyl - 5 - vinyl pyridine+0.75% of Complex IIc

Compositions A, B, E and F of the present invention and comparative compositions shown in the table were tested (I) in the Oldsmobile Scuffing Test under conditions described in the October 6, 1959, Report issued by Technical Committee B of ASTM Committee D-2 entitled "Engine Test Sequence for Evaluating Oils for API Service MS," and engine scuffing was visually rated as 1 to 10 with 10 being perfect and 1 being poor; (II) Exhaust Gas Rust Test (EGRT) which comprises exposing oil-dipped steel panels to the exhaust vapors of a single cylinder 4-cycle Briggs and Stratton engine oper-

ating on a high sulfur (1%) fuel. The panels are exposed to the hot exhaust gases for 30 minutes, then cooled to a temperature of 0° F. for 16 hours and allowed to warm to room temperature. The cycle is then repeated before inspection and rated on a scale of 1 to 10, where 1 is poor and 10 is perfect; and (III) GM-MS Test Sequences I-III under the following 1960 conditions:

*Engine test conditions*

| 10 | Hours                     | Sequence I                                        | Sequence II                                     | Sequence III       |
|----|---------------------------|---------------------------------------------------|-------------------------------------------------|--------------------|
|    |                           | 30 cycles,<br>10 min.<br>running,<br>50 min. down | 60 cycles,<br>3 hrs.<br>running,<br>3 hrs. down | 40 cycles          |
| 15 | R.p.m.                    | 3150±25                                           | 2500±20                                         | 1500±20            |
|    | Water out, ° F.           | 200±2                                             | 95±2                                            | 95±2               |
|    | Water in, ° F.            | 190 min.                                          | 85 min.                                         | 190 min.           |
|    | Oil temp., ° F.           | 280±2                                             | 120 max                                         | 120±2              |
|    | Loa <sup>1</sup> , B.H.P. | 30                                                | 0                                               | 25±2               |
|    | Air/fuel                  | 14.5±0.5                                          | 14±0.5                                          | 14±0.5             |
| 20 | Blow-by rate              | 0.4±0.1                                           | 0.8±0.1                                         | 2.0±0.2 c.f.m.     |
|    | Exhaust back              | 2±1 in.<br>water.                                 | 4±2 in.<br>water.                               | 20±4 in.<br>water. |

and the results were as follows:

TABLE I

|                                                                                                                                                                                                                            |                                                                   | Test                          |                                                              |     |
|----------------------------------------------------------------------------------------------------------------------------------------------------------------------------------------------------------------------------|-------------------------------------------------------------------|-------------------------------|--------------------------------------------------------------|-----|
|                                                                                                                                                                                                                            |                                                                   | I                             | II                                                           | III |
|                                                                                                                                                                                                                            | Oldsmobile<br>scuffing<br>test, visual<br>rating (10=<br>perfect) | EGRT<br>test (10=<br>perfect) | GM-MS<br>test, final<br>rating <sup>1</sup><br>(100=perfect) |     |
| 35 A                                                                                                                                                                                                                       | 9                                                                 | 9                             | 89                                                           |     |
| B                                                                                                                                                                                                                          | 9                                                                 | 9                             | 88.8                                                         |     |
| E                                                                                                                                                                                                                          | 9                                                                 | 9                             | 90                                                           |     |
| F                                                                                                                                                                                                                          | 8                                                                 | 8                             | 85                                                           |     |
| (1) Mineral lubricating oil plus<br>1% of dioleyl amide of<br>H <sub>2</sub> N—CH <sub>2</sub> CH <sub>2</sub> —N(C <sub>4</sub> H <sub>9</sub> )—<br>C <sub>12</sub> H <sub>25</sub> Cl <sub>2</sub> NH <sub>2</sub> (Ia) | 2 (1-2)                                                           | 3                             |                                                              |     |
| (2) Mineral lubricating oil plus<br>1% mixture of monoalkyl<br>dilauryl acid phosphate                                                                                                                                     | 2 (1-3)                                                           | 4                             | 90                                                           |     |
| (3) Mineral lubricating oil plus<br>2% 1-hydroxy ethyl-2-hepta-<br>decenyl imidiazoline plus 2%<br>nonyl phenoxy acetic acid                                                                                               | 2 (1-3)                                                           | 2                             | 75                                                           |     |
| (4) Mineral lubricating oil plus<br>4% 1-hydroxy ethyl-2-hepta-<br>decenyl imidiazoline                                                                                                                                    | 2 (1-3)                                                           | 2                             | 70                                                           |     |
| (5) Mineral lubricating oil plus<br>2% Ex. II copolymer                                                                                                                                                                    | 2 (1-3)                                                           | 1                             | 70                                                           |     |
| (6) Mineral lubricating oil                                                                                                                                                                                                | 4                                                                 |                               | 70                                                           |     |

<sup>1</sup> Mineral lubricating oil in 1-6=SAE 30.

<sup>2</sup> Bad scuffing.

Lubricating compositions of this invention are particularly applicable for high temperature, high speed use as in aviation engines, automotive engines and truck engines, as well as industrial equipment operating under the conditions described in this invention.

I claim as my invention:

1. A mineral lubricating oil composition consisting essentially of a major amount of mineral lubricating oil and from about 0.1% to about 10% each of an oil-soluble polymeric nitrogen-containing detergent selected from the group consisting of an oil-soluble copolymer of C-vinyl pyridine and a long chain alkyl methacrylate and an oil-soluble copolymer of N-vinyl pyrrolidone and a long chain alkyl methacrylate and an oil-soluble complex of a diamide having the formula



2. An acidic compound selected from the group consisting of a C<sub>1</sub>-18 alkyl acid phosphate and a C<sub>1</sub>-18 alkyl phenoxy carboxylic acid where R is a C<sub>8</sub>-22 alkyl radical, consisting of hydrogen and a C<sub>1</sub>-4 alkyl radical and n is an integer of 1 to 10.

3. A mineral lubricating oil composition consisting

essentially of a major amount of mineral lubricating oil and from about 0.1% to about 10% each of an oil-soluble copolymer of C-vinyl pyridine and a mixture of dissimilar long chain alkyl methacrylates and an oil-soluble complex of a diamide having the formula:



an a  $\text{C}_{1-18}$  alkyl acid phosphate where  $\text{R}$  is a  $\text{C}_{8-22}$  alkyl radical,  $\text{R}_1$  and  $\text{R}'$  are independently selected from the group consisting of hydrogen and  $\text{C}_{1-4}$  alkyl radical and  $n$  is an integer of from 1 to 10.

3. A mineral lubricating oil composition consisting essentially of a major amount of mineral lubricating oil and from about 0.1% to about 10% each of an oil-soluble copolymer of C-vinyl pyridine and a mixture of dissimilar long chain alkyl methacrylates and an oil-soluble complex of a diamide having the formula:



and a  $\text{C}_{1-18}$  alkyl phenoxy carboxylic acid where  $\text{R}$  is  $\text{C}_{8-22}$  alkyl radical,  $\text{R}_1$  and  $\text{R}'$  are independently selected from the group consisting of hydrogen and  $\text{C}_{1-4}$  alkyl radical and  $n$  is an integer of from 1 to 10.

4. A mineral lubricating oil composition consisting essentially of a major amount of mineral lubricating oil and from about 0.1% to about 10% each of an oil-soluble copolymer of C-vinyl pyridine and a mixture of dissimilar long chain alkyl methacrylates and an oil-soluble complex of dioleyl amide of



and a mixture of mono and dilauryl acid phosphate.

5. A mineral lubricating oil composition consisting essentially of a major amount of mineral lubricating oil and from about 0.1% to about 10% each of an oil-soluble copolymer of C-vinyl pyridine and a mixture of dissimilar long chain alkyl methacrylates and an oil-soluble complex of dioleyl amide of



and nonyl phenoxy acetic acid.

6. A mineral lubricating oil composition consisting essentially of a major amount of mineral lubricating oil and from about 0.1% to about 10% each of an oil-soluble copolymer of C-vinyl pyridine and a mixture of dissimilar long chain alkyl methacrylates and an oil-soluble complex of dioleyl amide of N-2-aminoethyl piperazine and a mixture of mono and dilauryl acid phosphate.

7. A mineral lubricating oil composition consisting essentially of a major amount of mineral lubricating oil and from about 0.1% to about 10% each of an oil-soluble copolymer of C-vinyl pyridine and a mixture of dissimilar long chain alkyl methacrylates and an oil-soluble complex of dioleyl amide of N-2-aminoethyl piperazine and nonyl phenoxy acetic acid.

8. A mineral lubricating oil composition consisting essentially of a major amount of mineral lubricating oil

and from about 0.1% to about 10% each of an oil-soluble copolymer of 2-methyl-5-vinyl pyridine and a mixture of lauryl and stearyl methacrylates and an oil-soluble complex of dioleyl amide of



and a mixture of mono and dilauryl acid phosphate.

9. A mineral lubricating oil composition consisting essentially of a major amount of mineral lubricating oil and from about 0.1% to about 10% each of an oil-soluble copolymer of 2-methyl-5-vinyl pyridine and a mixture of lauryl and stearyl methacrylates and an oil-soluble complex of dioleyl amide of



and nonyl phenoxy acetic acid.

10. A mineral lubricating oil composition consisting essentially of a major amount of mineral lubricating oil and from about 0.1% to about 10% each of an oil-soluble copolymer of 2-methyl-5-vinyl pyridine and a mixture of lauryl and stearyl methacrylates and an oil-soluble complex of dioleyl amide of N-2-aminoethyl piperazine and nonyl phenoxy acetic acid.

11. A mineral lubricating oil composition consisting essentially of a major amount of mineral lubricating oil and from about 0.1% to about 10% each of an oil-soluble copolymer of 2-methyl-5-vinyl pyridine and a mixture of lauryl and stearyl methacrylates and an oil-soluble complex of dioleyl amide of N-2-aminoethyl piperazine and a mixture of mono and dilauryl acid phosphate.

12. The composition of claim 8 containing from about 0.05% to 2% of bis(3,5-ditertbutyl-4-hydroxyphenyl)-methane.

13. The composition of claim 9 containing from about 0.05% to 2% of bis(3,5-ditertbutyl-4-hydroxyphenyl)-methane.

14. The composition of claim 10 containing from about 0.05% to 2% of bis(3,5-ditertbutyl-4-hydroxyphenyl)-methane.

15. The composition of claim 11 containing from about 0.05% to 2% of bis(3,5-ditertbutyl-4-hydroxyphenyl)-methane.

#### References Cited by the Examiner

| UNITED STATES PATENTS |       |                 |          |
|-----------------------|-------|-----------------|----------|
| 2,573,568             | 10/51 | Herman et al.   | 252-49.9 |
| 2,737,496             | 3/56  | Catlin          | 252-51.5 |
| 2,830,025             | 4/58  | Knowles et al.  | 252-52   |
| 2,843,548             | 7/58  | Westlund et al. | 252-51.5 |
| 2,914,968             | 7/60  | Hutchison       | 252-51.5 |
| 2,963,437             | 12/60 | Ries            | 252-49.8 |
| 3,100,749             | 8/63  | Wittner         | 252-49.9 |

#### FOREIGN PATENTS

|         |       |                |
|---------|-------|----------------|
| 159,789 | 11/54 | Australia.     |
| 760,554 | 10/56 | Great Britain. |
| 812,938 | 5/59  | Great Britain. |

60 DANIEL E. WYMAN, Primary Examiner.